

Jan. 12, 1932.

H. LOHmann

1,840,457

ALLOY

Filed Jan. 16, 1926



FIG. 1



FIG. 2



FIG. 3

Inventor  
Hugo Lohmann  
by  
Moritz Hause  
Attorney

## UNITED STATES PATENT OFFICE

HUGO LOHMANN, OF BERLIN-JOHANNISTHAL, GERMANY

## ALLOY

Application filed January 16, 1926, Serial No. 81,806, and in Germany January 24, 1925.

My invention relates to a new and improved method for making the carbides of the relatively infusible metals.

One of the objects of my invention relates 5 to a new and improved method for making tungsten carbides. This tungsten carbide may contain molybdenum. The process also applies to making a molybdenum carbide. Tungsten and molybdenum are generally referred to as heavy metals, because their 10 atomic weights are respectively 184 and 96. Hence, whenever I refer to a tungsten carbide or a tungsten alloy, either in the description or in the claims, it is to be understood that 5 this includes a similar molybdenum alloy, or an alloy containing both tungsten and molybdenum.

Another object of my invention is to provide a new and improved method for producing 20 hard and strong masses or bodies of the carbides above mentioned so that these masses or bodies can be utilized for various mechanical purposes, such as, for example, for manufacturing tools.

25 Another object of my invention is to provide carbides of the relatively infusible metals and in particular a tungsten carbide in which the carbon is present in proper proportion.

30 Other objects of my invention will be set forth in the following description and drawings which illustrates a preferred embodiment thereof, it being understood that the above general statement of the objects of my 25 invention is intended merely to generally explain the same and not to limit it in any manner.

Fig. 1 is a diagrammatic side view, partially in section, showing a carbon tube fur- 40 nace.

Fig. 2 is an end view of the device shown in Fig. 1.

Fig. 3 is a diagrammatic view showing the boat and casting mold.

45 Methods have been known for many years for making hard and strong articles composed of the carbides of the relatively insoluble metals, such as tungsten carbide.

50 According to these previously known methods, the metallic carbides were first manufac-

tured by a melting process, they were then powdered and were then subjected to a second heat treatment with or without the addition of other substances. In this second heat treatment, the temperature of the mass was raised 55 either to the melting point or almost up to the melting point. This method included two steps and had many disadvantages and it was not reliable, so that the products resulting therefrom were often worthless. In addition, 60 it required the careful attention of highly skilled workmen.

According to my invention, I utilize a mixture of an oxygen compound of the metal, together with an additional metal or metallic 65 compound, the melting point of said additional metal or metallic compound being as close as possible to the melting point of the first mentioned metal. This mixture is melted in the presence of carbon and is cast in molds, 70 the melted mass being removed as quickly as possible from the furnace or heated space, to prevent an undesirable excess saturation of the product with carbon. This causes the excess carbon to be separated when the molten 75 mass solidifies.

For example, an oxygen compound of the infusible metal, as, for example, tungstic acid or the anhydride, or highly reduced powdered metallic oxides, such as, for example, 80 reduced metals which still contain a substantial proportion of oxygen can be mixed with a heavy metal or a compound thereof, such as, for example, thorium or uranium oxide or tantalum or a similar metal or metallic 85 oxide. These additional metals also have high atomic weights and high melting points. Thus the atomic weight of thorium is 232.4, that of tantalum is 181.5, and that of uranium is 238.5. While my invention generally 90 relates to produce a dense, homogeneous alloy consisting of tungsten, carbon, and a metal whose atomic weight is not less than that of tantalum (such as thorium), it is not restricted to an absolutely pure alloy. As above 95 mentioned, these additional metals or metallic oxides have melting points which are the same or which are substantially the same as the metal whose carbide is to be formed. The mixture made as above specified is formed 100

into a briquette by pressure. This briquette is now preferably heated in carbon vessels to which the molds are directly joined, in inclined carbon tube ovens until the desired 6 reaction and melting temperature is attained. The carbon of which the vessels are made, as well as the carbon-containing gases present in the furnace or heated space, first reduces the metallic oxide or oxides to the metallic 10 form when the proper reaction temperature has been attained, and then produces the formation of the metallic carbide. At the moment when the carbide is melted and for a short time thereafter, the metallic carbide 15 has the desired proportion of or saturation with the carbon. The melted mass flows immediately into the associated mold and fills the mold. It is desirable to remove the mold together with the molten contents thereof 20 out of the oven as soon as possible.

As shown in Figs. 1 and 2, a carbon tube furnace may be used having graphite electrodes *a* connected to buss bars. A carbon tube *b* is also provided and the material to be 25 treated is put into a boat *d*.

As shown in Fig. 3, the boat *d* in which the material is melted may have a metal body *f* and it may be connected to a casting mold *e*.

I have discovered that if the metal is subjected for a substantial period to the action 30 of the carbon while the said metal is in the molten form, that the mixture is supersaturated with the carbon, and above the limit desired. If the molten mass is quickly removed from the oven, the excess carbon in the 35 form of graphite is separated when the mass solidifies. The amount of carbon present in the carbide made according to my invention is between 4½% to 5%. For example, if the 40 carbide of tungsten is prepared according to my invention, an alloy is produced which has very desirable properties. The use of tantalum (or of tantalum oxide, which is an equivalent) produces a particularly useful alloy.

If instead of employing the oxides of the infusible metals as in the example above given, the pure metal or the metal in the commercial form is utilized (such as tungsten, for example), it is not necessary to reduce 45 the raw material so that the process can be carried out much more quickly. However, the reactions are substantially the same as those above described.

I have discovered that when thorium carbide is mixed with tungsten and the mixture is melted in the retorts, that very hard and mechanically firm bodies are produced which have an absolutely homogeneous structure, especially if a small amount of molybdenum is 55 added to the mixture. The thorium carbide can contain from 12% to 14% of carbon. Hence, the carbon for producing the tungsten carbide is partially secured from the thorium carbide mixed therewith as above 60 specified.

When this mixture is melted (as for example, the mixture of tungsten and thorium carbide) the thorium carbide at once yields some of the carbon to the other metal, such as tungsten, which is substantially free from carbon. Likewise, the tungsten takes up some of the carbon of the vessel. The alloy then contains from 4½% to 5% of carbon. 70

The pouring of the molten mass can take place as above specified. In carrying out my process, it is preferable to use 100 parts by weight of solid raw tungsten, 5 to 10 parts by weight of thorium carbide, and 3 to 5 parts by weight of molybdenum. 75

Unsaturated thorium carbide, which is present in the mixture, makes it extremely hard and tough, which are decided advantages. If the tungsten contains some oxygen, then the thorium carbide simultaneously reduces the oxide which is present to the metallic state. 80 85

I have shown a preferred embodiment of my invention, but it is clear that numerous changes and omissions could be made without departing from its spirit. 90

#### Claims:

1. As a new article of manufacture, a dense and homogeneous alloy consisting substantially of tungsten, carbon, and tantalum, the tungsten comprising the major portion of the alloy, and the percentage of carbon being not less than four per cent. 95

2. As a new article of manufacture, a dense and homogeneous alloy consisting substantially of tungsten, carbon, tantalum and molybdenum, the tungsten comprising the major ingredient of the alloy, and the percentage of carbon being not less than four per cent. 100 105

In testimony whereof I affix my signature.  
HUGO LOHMAN.

110

115

120

125

130